

Nov. 17, 1931.

D. E. WEBSTER

1,832,515

ABRASIVE ARTICLE

Filed March 16, 1931

FIG. 1



FIG. 2



WITNESSES

Franklin E. Johnson  
W R Greenwood

INVENTOR

DUANE E. WEBSTER

BY  
Clayton L. Jenkins  
ATTORNEY

## UNITED STATES PATENT OFFICE

DUANE E. WEBSTER, OF WORCESTER, MASSACHUSETTS, ASSIGNOR TO NORTON COMPANY,  
OF WORCESTER, MASSACHUSETTS, A CORPORATION OF MASSACHUSETTS

## ABRASIVE ARTICLE

Application filed March 16, 1931. Serial No. 523,002.

My invention relates to grinding wheels and more particularly to a ring wheel for use in a disk grinding machine in which it is supported to provide an annular, plane 5 grinding surface.

One type of grinding wheel for this purpose comprises a metal backing disk to the end face of which a suitable grinding member, of granular abrasive material bonded 10 by an organic or vitrified ceramic bond, is secured by a cementitious material, such as shellac or resin cement and the like. Suitable devices, such as projecting studs, are provided in the backing disk for attaching 15 the wheel to a metal supporting disk carried by a rotatable driving shaft. Heretofore, in the manufacture of wheels of this type, it is not uncommon to find that the grinding member has become loose from its metal 20 backing or that serious structural cracks and ruptures have formed in the abrasive body itself. It is found that these defects ordinarily occur when the assembled wheel is removed, while hot, from the baking oven 25 in which the resinous cement has been subjected to a heat hardening operation. On cooling to room temperature, stresses are produced in the warm mass, due to shrinkage or the like, which arise from the great difference 30 in the coefficients of expansion of the abrasive bond and the metal constituting the support for the grinding member. Even if not badly cracked when initially manufactured, these fragile grinding members 35 may be defective and later break during the grinding operation while the wheel is in use. Such breakage may mean a considerable loss to the user, hence every effort has been made to prevent the occurrence of such extreme 40 thermal stresses, but due to difficulties inherent in the processes of manufacture and the natural physical properties of the materials which must be considered, it has not been found possible to do so at all times.

45 It is accordingly an object of my inven-

tion to overcome such difficulties and to provide a grinding wheel construction which is capable of being easily manufactured and will not develop such detrimental defects.

A further object of my invention is to employ a wheel construction in which the parts will be integrally united to form a unitary body whereby the thermal changes due to expansion and contraction will be evenly and uniformly distributed throughout. 55

In accordance with my invention I propose to make an abrasive article, such as a grinding wheel, in the form of a composite or laminated structure in which an abrasive body composed of granular abrasive material combined with an organic bond, such as a synthetic resin or resinoid, is integrally united with a self-supporting backing of a hard, unyielding, organic composition which comprises substantially the same material as 60 the wheel bond and the backing and has substantially the same coefficient of expansion. In my preferred form the backing 65 comprises a resinoid body, which may be reinforced by a strengthening member embedded therein, and an abrasive body of resinoid bonded abrasive grains united to form a unitary body. The backing and abrasive may be formed integrally in a single 70 operation without an intermediate body of cement or the two parts may be initially molded separately and then united by a cement. In either case, the bond, backing 75 and cement will have substantially the same coefficients of expansion and will preferably 80 comprise the same resinoid. As one manner of carrying out this invention, I make use of a synthetic resin of the phenolic condensation type as is obtained by the reaction of phenol or its homologues with formaldehyde and which is capable of being converted 85 to form an unusually tenacious bond when sufficiently heated to produce the final reaction.

90 In the drawings which illustrate one em-

bodiment of this invention and in which like reference numerals indicate like parts:

Fig. 1 is a plan view of a grinding wheel embodying my invention; and

Fig. 2 is a sectional view, taken on the line 2—2 of Fig. 1, of the assembled wheel when ready for use.

As illustrated, the abrasive body may be made up in accordance with standard practice, such as disclosed in the patent to Brock No. 1,537,454 of May 12, 1925, of a pre-formed abrasive annulus or ring 10 having a plane grinding surface 11 and composed of granular abrasive material, such as crystalline alumina or silicon carbide, bonded by a synthetic resin composed of a heat hardening condensation product, such as one of the type commonly known under the trade-mark "Bakelite". Hereafter, these resin condensation products will be referred to as "resinoids", so designated in the art on account of their characteristic difference from the properties common to the natural resins in that they polymerize and harden upon heating to a form that is hard, infusible and insoluble.

In order to support the abrasive annulus rigidly so that it may be mounted directly on the end of a rotating shaft, I provide a backing support for the wheel which is integrally united to the grinding ring so as to form a unitary grinding body. The type of backing support shown in the drawings comprises a disk 15 having a reticulated reenforcement therein, which possesses sufficient strength and rigidity to support the abrasive annulus during the grinding operation and is adapted to be mounted on a rotating shaft (not shown) by means of an outer hub 16. In my preferred construction the disk 15 may be made of a material commonly known under the trade-mark "Micarta", which comprises a preformed molded body made up of layers of fabric or other reenforcing material of suitable thickness which is cut to the desired shape, and then impregnated with a resinoid binding media, more particularly a phenolic resin, such as "Bakelite" resin. The impregnated material is then subjected to heavy pressure by which the various sections are intimately joined together as well as shaped, after which it is subsequently baked to harden the resin. The backing member, when completed, will constitute the sole support for the wheel structure and will be directly mounted upon the rotatable driving spindle.

To this end, the hub 16 is provided with an exterior surface of the proper size and of the required shape to fit within and be clamped against the inner peripheral surface of a suitably shaped collar (not shown) adapted to support the wheel on the rotating shaft. The disk 15 is provided with a central aperture 18 adapted to fit over the end portion of the rotatable shaft. In close proximity to this aperture there are provided a

series of holes 20 adapted to receive suitable clamping screws or bolts which may pass through the backing disk and into the collar to thereby fasten the grinding wheel to the shaft.

In order that the grinding ring may fit properly against the backing disk, the outer surface of the abrasive face opposed to the disk is provided with a hub portion 22 which is of the proper size to fit within a correspondingly shaped depression or cavity 23 formed in the opposed face of the backing disk 15. When assembled, the interfitting faces of the annulus and the backing disk respectively provide the opposed surfaces with a large area of contact and thus enable the parts to be more firmly united by the securing medium.

While the grinding ring may be formed in situ on the backing after the latter has been fully made, or the two parts may be molded of the "green material" and all of the resinoid be heat set in a single operation, yet in my preferred form the abrasive annulus and the backing are first initially made in separate operations and then cemented together. To this end, I propose to place a layer of a suitable cementitious organic material 25 between the juxtaposed faces of the abrasive ring and the backing disk which when matured will hold the parts integrally together. A suitable cement for this purpose is a composition in which the bonding vehicle embodied therein is of the same type as that incorporated within the wheel structure and its backing member. To this end, the cement may comprise a mixture of a resinoid, such as "Bakelite", and a suitable plasticizing agent, such as furfural, acetone, etc., the latter being employed in amounts sufficient to produce a mass of the desired plasticity.

Upon the application of heat, the composition will react to form an infusible, insoluble condensation product with the annulus and its backing disk integrally joined together to form a unitary inflexible grinding body. In practice, the cement layer may be applied to the bonding face of either the preformed annulus or the backing disk, prior to their assembly. The parts are thereafter assembled and the structure subsequently heat treated at a temperature sufficient to mature the resinous material.

In order that the grinding ring may be more securely and intimately held to the backing disk by the resinous layer, the disk may be provided with a series of holes 30 which extend through the disk and are countersunk on the back face so as to appear as an inverted frustum of a cone, the small end of which is adjacent to the juxtaposed face of the grinding annulus. On assembly of the parts, the layer of resin cement will flow into and fill the countersunk holes, thus forming a series of tapered or frusto-conical dow-

els of the resinous material which integrally unites and bonds with the disk during the final baking operation.

It will of course be understood that the parts may be united in any other desired manner. For example, it is feasible, after placing a preformed backing disk in a mold, to coat the bonding face of the disk with the resin cement and then mold an abrasive annulus thereto from a suitable mixture of abrasive grains and the "Bakelite" resin powder under heat and pressure. The article may then be removed from the mold and thereafter baked to mature the resin. Likewise, the cement layer may be omitted, and the resinoid bond used with the abrasive grains will unite the parts integrally. In that case the mixture of abrasive grains with resinoid bond, and a plasticizing medium, such as furfural, may be placed on the preformed "Micarta" backing and the parts then pressed and heat hardened. The abrasive body and associated parts may be made in accordance with standard practice, such as that described in the patent to Martin No. 1,626,246 of April 26, 1927.

This type of grinding wheel possesses a marked advantage over one made of other materials which have heretofore been employed for such purposes. The various portions of the wheel structure are made of the same type of bond which, when matured, results in a unitary structure integrally united by a single tenacious bond. The difference of coefficient of expansion between the various parts is diminished substantially to zero value by the proper selection of the bonding ingredients used, and the structure will accordingly be free from the strains which such differences set up when the article is subsequently heated or cooled. By so constructing such a wheel to prevent serious losses due to breakage and rupture, I have made it feasible to manufacture the ring wheel more successfully and to a greater extent than heretofore obtainable.

While I have specifically described my invention as adapted to the manufacture of an abrasive wheel of a phenolic resin composition it will be obvious to those skilled in the art that other abrasive articles in which the same or similar properties are desired may be made and that other materials may also be used throughout the structure to suit the particular conditions which may in the case be involved. Such modifications or substitutions of my invention as lie within the scope of the appended claims are, however, to be considered as embodied in the above specification.

Having thus described my invention, what I claim as new and desire to secure by Letters Patent is:

1. A grinding wheel comprising an abrasive body of abrasive grains containing a

resinoid bond uniting the grains into a unitary mass and a rigid reenforcing backing therefor comprising a resinoid integral with the bond of the abrasive body, said backing being the sole support for the abrasive body and directly mounted upon a rotatable driving spindle. 70

2. A grinding wheel comprising an abrasive body of abrasive grains containing a resinoid bond uniting the grains into a unitary mass and a backing therefor, which comprises a rigid resinoid body and which is integral with and has substantially the same coefficient of expansion as the bond of the abrasive body. 75

3. A grinding wheel comprising an abrasive body of abrasive grains containing a resinoid bond uniting the grains into a unitary mass and a backing therefor, which comprises a rigid resinoid body containing layers of reenforcing material, and which is integral with the bond of the abrasive body, said body and the backing each having substantially the same coefficient of expansion. 80

4. An abrasive article comprising a resinoid body, an abrasive member of resin bonded abrasive grains, and a layer of cementitious organic material between and integrally uniting the bonded abrasive member with said resinoid body. 85

5. An abrasive wheel comprising a rigid resinoid body containing reinforcing layers of reticulated material and an abrasive member of bonded abrasive grains integrally united thereto and having an abrading surface. 90

6. An abrasive wheel comprising a rigid non-abrasive resinoid body and an abrasive member of resin bonded abrasive grains having an end face opposed to said body and integrally united therewith, the opposite end face of said abrasive member providing a plane grinding surface for the wheel. 95

7. A laminated abrasive article having an abrading facing of phenolic resin bonded abrasive grains, a hard resinoid backing layer, and an intermediate layer of cementitious material matured therebetween and integrally uniting said facing and the backing. 100

8. An abrasive wheel comprising an abrading body of phenolic resin bonded abrasive grains, a rigid resinoid backing support therefor containing reenforcing layers of fabric, and a cementitious medium between and integrally uniting said backing support and the abrading body embodying a resinoid substantially identical with that contained in the abrading body and the backing support. 105

9. A composite grinding wheel comprising an abrading body of resinoid bonded abrasive grains, a rigid backing of resinoid material, and a layer of cementitious resinoid material therebetween and integrally uniting said body and backing to form a unitary rigid grinding structure in which the resinoid for

the various portions has substantially the same coefficient of expansion.

10. A grinding wheel comprising a grinding annulus of resinoid bonded abrasive grains, a rigid support therefor of disk-like shape containing a resinoid and integrally united to said annulus, and means central with said support which constitutes the sole rotatable support of the wheel structure during grinding.

Signed at Worcester, Massachusetts this 13th day of March 1931.

**DUANE E. WEBSTER.**

15

20

25

30

35

40

45

50

55

60

65